

Feb. 14, 1950

N. C. GEORGE ET AL  
MANUFACTURE OF TIN PLATE

2,497,164

Filed June 25, 1946

FIG. 1.



FIG. 2.



*Inventors:*  
NELSON C. GEORGE and  
ROLF C. HAAB,  
by: Donald G. Dalton  
their Attorney.

## UNITED STATES PATENT OFFICE

2,497,164

## MANUFACTURE OF TIN PLATE

Nelson C. George, Crown Point, and Rolf C. Haab,  
Gary, Ind., assignors to Carnegie-Illinois Steel  
Corporation, a corporation of New Jersey

Application June 25, 1946, Serial No. 679,305

2 Claims. (Cl. 148—12)

1

This invention relates to the manufacture of tin plate, and more particularly to the improvement of the drawing properties thereof.

In the shaping of cold-reduced tin plate to form various articles considerable difficulty is experienced in eliminating defects caused by uneven drawing of the metal. This results in a drawn article of abnormal dimensions. That is, the drawn article at certain points will be of proper dimensions or, even undersized, while at other points the dimensions will be so increased as to produce what are known as "ears." In the manufacture of bottle caps, for example, extreme cases of uneven drawing necessitate the use of a shell with a serrated edge to assure firm holding of the inside washer on curling; whereas a smooth-edged shell is much more preferable, of course, to minimize the exposure of the steel on the cut edge and thereby reduce the possibilities of internal rusting. When the bottle caps are formed with serrated edges, the uneven drawing, or "earing," manifests itself in uneven teeth or serrations, the same being readily perceived when two bottle caps are placed in opposition.

Numerous attempts have been made to definitely ascertain the cause of uneven drawing, or "earing." Our investigations have shown that in order to eliminate or materially reduce tendencies toward uneven drawing, it is necessary to maintain close gage tolerance, uniform hardness, and uniform grain structure from the edge of the tin plate to the center thereof; and also that mechanically capped steel is for these purposes to be preferred over rimmed or killed grades.

Among other factors influencing the behavior of the tin plate during drawing is that of crystal anisotropy, and it involves numerous problems since present day microscopic study does not reflect preferred orientation in the shape of the grains composing the metal.

Our experiments regarding the question of crystal orientation involved investigation of the magnetic torque characteristics of the tin plate. A satisfactory method of investigating magnetic torque characteristics may be practiced by utilizing a simple apparatus comprising a rotatable magnetic field in which a disk-shaped test-piece is suspended on a wire having predetermined mechanical torque characteristics. Rotating the magnetic field through 360° brings forth the tendency of the test disk to align itself with the field, and the amount of torque induced by the alignment can be measured in units of force by determining the degree of suspension-wire twist. The number of dynes per square centimeter divided by 1000 is a convenient variable for expressing the magnetic torque observed. Plotting this number against the angle of rotation of the test disk generates curves characteristic of anisotropy of the test specimens. The reversals

2

and the peak magnitudes of the curve resulting from plotting the rotation of the magnetic field versus the induced torsional force indicate the degree of preferred orientation of the specimen.

Since the rotation of the test-pieces causes a type of phenomena which may be held as substantially recurrent, the curves produced apparently correspond to waves.

We have discovered that satisfactory tin plate is characterized by generating a magnetic torque curve of substantially sinusoidal shape which is substantially free from harmonics; and that tin plate having uneven drawing characteristics is characterized by generating a magnetic torque curve of sinusoidal shape which includes harmonics. When the magnetic torque curve is free from harmonics, the tin plate has random crystalline orientation; when harmonics are present, the tin plate has preferred orientation which is undesirable for our purposes.

According to the teaching of the present invention there is correlation between the magnetic torque test results and the response to fabricating practice including the grade of steel, the steel making practice, the hot-rolling methods, temper-rolling procedures, and influences in gage variation. None of the aforementioned factors is alone responsible for the peculiar behavior of sheets, but the present invention teaches that uneven drawing and the defect known as "earing" can be eliminated by a specific combination of variables, as will appear more fully hereinafter.

The invention, then, comprises the features hereinafter described and as particularly pointed out in the claims, the following description and the annexed drawings setting forth in detail certain illustrative embodiments of the invention, these being indicative of several of the number of ways in which the principles of the invention may be employed.

In said drawings:

Figure 1 is an elevation of two pairs of superposed bottle caps, the pair at the left, designated as "A," representing articles which are practically entirely free from the condition known as "earing"; while in the right-hand pair of bottle caps, designated as "B," earing is so marked as to render them unacceptable to the trade; and

Figure 2 is a chart illustrating the magnetic torque in dynes per  $CM^2 \times 10^{-3}$ ; and from which it will be noted that the curve "A" is substantially sinusoidal and substantially free from harmonics, while the curve "B" includes harmonics.

In accordance with the teachings of the present invention there is produced a low carbon (.12% maximum carbon) steel which is hot-rolled into strip, coiled, pickled, cold-reduced, annealed, temper-rolled, and tinned by a com-

bination of steps which are individually old.

The composition of the steel of the present invention is approximately within the following ranges:

|                                       | Percent       |
|---------------------------------------|---------------|
| Carbon                                | 0.030 to 0.15 |
| Manganese                             | 0.60 maximum  |
| Phosphorus                            | 0.150 maximum |
| Sulphur                               | 0.050 maximum |
| Silicon                               | 0.010 maximum |
| Copper                                | 0.30 maximum  |
| and the remainder substantially iron. |               |

A preferred embodiment comprises a steel the composition of which is approximately within the following ranges:

|            | Percent       |
|------------|---------------|
| Carbon     | 0.05 to 0.08  |
| Manganese  | 0.30 to 0.45  |
| Phosphorus | 0.12 maximum  |
| Sulphur    | 0.035 maximum |
| Silicon    | 0.010 maximum |
| Copper     | 0.20 maximum  |

The steel of the invention is teemed into 30" x 48" ingot molds, mechanically capped with the capping time not longer than 3 minutes, and 30 seconds being preferable. The steel so capped is hot-rolled in steps to strip of approximately 0.080 inch thickness and the strip rolling is finished at a minimum temperature of approximately 1580° F. The strip so produced is coiled at a minimum temperature of 1300° F., then continuously pickled in sulphuric acid, cold-reduced from substantially 0.080 inch to substantially 0.0110 inch, electrolytically cleaned, box annealed in a controlled atmosphere to deoxidize at between approximately 1200° F. and approximately 1280° F., the following atmosphere being preferable: approximately 4% CO<sub>2</sub>, approximately 9.5% CO, approximately 16% H<sub>2</sub>, approximately 1.2% CH<sub>4</sub>, approximately 71.2% N, dew point between approximately -40° and approximately +80° F. The annealed strip is temper-rolled approximately 4%, and electrolytically coated with approximately 0.5 lb. of tin per base box. If the foregoing minimum finishing and coiling temperatures are not maintained, the random crystalline orientation, which is necessary for a non-earing tin plate, is lost. The magnetic torque curve furnishes a ready test for such orientation.

We have discovered that tin plate made in substantial accordance with the practice described immediately hereinbefore possesses properties expected of a high quality commercial tin plate, namely Rockwell 30 T. hardness of 54/60, grain size showing absolute values of 7 to 9 equiaxed grains, elongation of 15 to 25% in two inches, yield point of 38,000 to 42,000 pounds per square inch, tensile strength of 43,000 to 49,000 pounds per square inch; and in addition is characterized by sinusoidal magnetic torque curve devoid of harmonics. This steel is further characterized by being practically entirely free from tendency toward uneven drawing, or "earing."

While we have shown and described certain specific embodiments of the present invention, it will be readily understood by those skilled in the art that we do not wish to be limited exact-

ly thereto, since various modifications may be made without departing from the scope of the invention as defined in the appended claims.

We claim:

1. In the manufacture of cold reduced steel strip for tin plating and subsequent deep drawing of symmetrical shapes, wherein capped steel of approximately the composition:

|            | Percent       |
|------------|---------------|
| Carbon     | 0.030 to 0.15 |
| Manganese  | 0.60 maximum  |
| Phosphorus | 0.150 maximum |
| Sulphur    | 0.050 maximum |
| Silicon    | 0.010 maximum |
| Copper     | 0.30 maximum  |

and the balance iron and incidental impurities, is hot rolled into strip, the hot rolled strip is coiled, pickled and cold reduced, and the cold reduced strip is annealed at approximately 1100° F. to 1300° F., a method of producing random crystalline orientation in the steel as measured by its magnetic torque characteristics which, when expressed in a sinusoidal curve, are practically entirely free of harmonics, and thereby of preventing earing when the steel is drawn, comprising finishing the hot rolling at a temperature above 1580° F. and performing the coiling at a temperature above 1300° F.

2. In the manufacture of cold reduced steel strip for tin plating and subsequent deep drawing of symmetrical shapes, wherein steel of approximately the composition:

|            | Percent       |
|------------|---------------|
| Carbon     | 0.030 to 0.15 |
| Manganese  | 0.60 maximum  |
| Phosphorus | 0.150 maximum |
| Sulphur    | 0.050 maximum |
| Silicon    | 0.010 maximum |
| Copper     | 0.30 maximum  |

and the balance iron and incidental impurities, is hot rolled into strip, the hot rolled strip is coiled, pickled and cold reduced, and the cold reduced strip is annealed at approximately 1100° F. to 1300° F., a method of producing random crystalline orientation in the steel as measured by its magnetic torque characteristics which, when expressed in a sinusoidal curve, are practically entirely free of harmonics, and thereby of preventing earing when the steel is drawn, comprising finishing the hot rolling at a temperature above 1580° F. and performing the coiling at a temperature above 1300° F.

NELSON C. GEORGE.  
ROLF C. HAAB.

#### REFERENCES CITED

The following references are of record in the file of this patent:

#### UNITED STATES PATENTS

| Number    | Name            | Date          |
|-----------|-----------------|---------------|
| 1,994,276 | Graham et al.   | Mar. 12, 1935 |
| 2,264,266 | Jacobs et al.   | Nov. 25, 1941 |
| 2,309,801 | Veeder          | Feb. 2, 1943  |
| 2,377,922 | Campbell et al. | June 12, 1945 |

#### OTHER REFERENCES

- 70 "The Making, Shaping, and Treating of Steel," 5th ed., pp. 1277-1283, by Camp & Francis. Carnegie-Ill. Steel Corp., Pitts., Pa., 1940.

**Certificate of Correction**

Patent No. 2,497,164

February 14, 1950

NELSON C. GEORGE ET AL.

It is hereby certified that error appears in the printed specification of the above numbered patent requiring correction as follows:

Column 3, line 20, for "0.12 maximum" read *.012 maximum*;  
and that the said Letters Patent should be read with this correction therein that the same may conform to the record of the case in the Patent Office.

Signed and sealed this 30th day of May, A. D. 1950.

[**SMAL**]

THOMAS F. MURPHY,  
*Assistant Commissioner of Patents.*